

# United States Patent Office

2,802,715

Patented Aug. 13, 1957

1

2,802,715

**PROCESS FOR THE BOILING-OFF AND BUCKING OF CELLULOSE FIBERS IN AQUEOUS ALKALINE SOLUTION CONTAINING R-(OC<sub>2</sub>H<sub>4</sub>)<sub>n</sub>OCH<sub>2</sub>COOM COMPOUNDS**

Kurt Hofer, Neue Welt, near Basel, and Hans Henmi, Binningen, near Basel, Switzerland, assignors, by mesne assignments, to Saul & Co., Newark, N. J., as nominee of Fidelity Union Trust Company

No Drawing. Application May 3, 1954,  
Serial No. 427,366

Claims priority, application Switzerland May 6, 1953

10 Claims. (Cl. 8—139)

The present invention is concerned with the cleaning of cellulose fibers as for example those in the so-called gray state, more especially by boiling-off and bucking.

A primary object of the invention is the embodiment of a cleaning process of the character aforesaid, whereby the boiling-off and/or bucking may proceed in more efficient manner and whereby the treated fibers are better suited for subsequent treatments, such as mercerization, bleaching, dyeing, finishing and the like.

This object is realized according to the present invention, briefly state, by subjecting the cellulose fibers to treatment at temperatures above 75° C. in an alkaline bath containing polyether carboxylic compound corresponding to the formula



wherein R stands for a saturated or unsaturated aliphatic hydrocarbon radical with 8 to 20 carbon atoms or for an alkylaryl or hydrogenated alkylaryl radical with 8 to 25 carbon atoms, n is a whole number which is greater than 1, and M represents a cation.<sup>1</sup> Cellulose fibers thus created become highly wettable and do not lose this property upon being rinsed or washed, boiled, mercerized or bleached. Accordingly, upon the further treatment of such fibers in aqueous media wherein good wetting and penetration normally requires the addition of a wetting agent, it is possible according to the present invention successfully to carry out such further treatment without having to add a wetting agent.

The thus-realizable rapid wettability makes it possible to carry out mercerizing, bleaching, dyeing, finishing and the like processes more quickly and more uniformly. Moreover, the presence of a compound of Formula I facilitates the penetration of the boiling-off and bucking liquors into the fibers, so that the boiling-off or bucking process proceeds more rapidly and more uniformly.

This property of the aforesaid polyether carboxylic acid compounds (I) is surprising, since it cannot be realized at all or only to a greatly diminished extent with the known bucking assistants such as the alkylaryl sulfonates, the alkyl sulfates, the fatty acid condensation products, etc.

Illustrative of compounds of Formula I which are particularly useful in carrying out the present invention are the following compounds:



2



and their water-soluble salts, such as their sodium and potassium salts. These compounds can be prepared in known manner for example from the corresponding polyglycol ethers and chloroacetic acid.

15 The compounds (I) can be used alone or in combination with other known bucking agents. Because of their good solubility and stability in alkaline medium, even at high temperatures, the said compounds (I) are particularly useful in the aforesaid bucking and boiling-off of cellulose fibers.

20 The following illustrative examples set forth presently-preferred exemplary embodiments of the invention

*Example 1*

25 A cotton cretonne fabric, directly as it comes from the loom, is boiled-off for two hours in an aqueous caustic soda liquor of 2° Bé. strength in a goods to liquor ratio of 1:40 in an open vessel in the presence in the liquor of one gram of sodium oleyl-dodecaglycoloxyacetate



30 per liter of liquor, after which the material is washed with hot water and then with cold water until it is neutral, whereupon it is dried at 60° C. The material then has an excellent wettability in aqueous medium, which is not the case if the boiling-off is carried out in the absence of the said compound.

*Example 2*

35 Unboiled cotton is boiled-off for two hours in an aqueous caustic soda liquor of 2° Bé. strength in a goods to liquor ratio of 1:40 in the presence in the liquor of one gram of sodium oleyl-dodecaglycoloxyacetate per liter of liquor, after which the material is washed with hot water and then with cold water until it is neutral, whereupon it is dried. After this treatment, the material has an excellent absorptive action.

*Example 3*

40 Gray cotton pearl yarn 3/2 is boiled-off in an aqueous caustic soda liquor of 2° Bé. strength in a goods to liquor ratio of 1:40 for one and one-half hours in an open vessel in the presence in the liquor of one gram per liter of sodium oleyl-dodecaglycoloxyacetate, after which the material is washed neutral and dried. By way of comparison, a similar yarn is boiled-off in an aqueous caustic soda liquor of 2° Bé. strength in the same bath ratio for 4 hours with no addition to the liquor. If these yarns are now subjected to comparative shrinking tests in caustic soda of 30° Bé. strength at 20° C., then the yarn which was boiled-off without the addition of assistant shows after 90 seconds a shrinking of 12.2%, while that which was boiled-off with the assistant shows a shrinkage of 22%.

*Example 4*

45 Gray cotton pearl yarn 3/2 is boiled-off for one and one-half hours in an aqueous caustic soda liquor of 2° Bé. strength, containing one gram of sodium lauryltetraglycoloxyacetate [C<sub>12</sub>H<sub>25</sub>O(CH<sub>2</sub>CH<sub>2</sub>O)<sub>4</sub>CH<sub>2</sub>COONa] per liter of liquor, in an open vessel. If this yarn is subjected to a comparative test, after the manner set forth in Example 3, with a like yarn which was boiled-off un-

<sup>1</sup> By the recitation that "n is a whole number greater than 1" is meant that n may range from as low as 2 to as high as 20.

der the same conditions but in the absence of the added assistant, it will be found that the yarn treated with the assistant shrinks to an extent of 21.4% in 90 seconds while that boiled-off without the assistant shrinks only to an extent of 14.6%.

*Example 5*

Cotton pearl yarn 3/2 in the gray is boiled-off for 2 hours in an aqueous caustic soda liquor of 2° Bé. strength, containing one gram of sodium iso-octylphenyl- or iso-octylhexahydrophenyloctaglycoloxyacetate per liter of liquor, in an open vessel. The material is thereupon rinsed and dried. Shrinkage measurements according to Example 3 show that, in contrast to the yarn which was boiled-off without the added assistant and which shrinks only about 12.8% under the given conditions, the yarn which was boiled-off with the assistant shrinks to an extent of 21.3% in the same time (90 seconds).

*Example 6*

A piece of unboiled cotton cretonne is bucked for two hours in an aqueous caustic soda liquor of 2° Bé. strength under a pressure of one and one-half atmospheres in the presence in the liquor of 0.25 gram of sodium oleyldeca-glycoloxyacetate with a goods to liquor ratio of 1:10. The material is then washed and dried. The thus-treated piece of fabric wets very easily, while a similar piece of fabric which was bucked as above but without the assistant shows only a very slight wettability.

*Example 7*

A piece of cotton cretonne, as it comes from the loom, is boiled-off for two hours in an aqueous caustic soda liquor of 2° Bé. strength in a goods to bath ratio of 1:40 in an open vessel with the addition to the liquor of one gram per liter of sodium lauryl-hexaglycoloxyacetate, after which the material is rinsed until it has a neutral reaction and is then dried. This treatment imparts outstanding wettability to the material.<sup>1</sup>

*Example 8*

A piece of cotton cretonne fabric is bucked for two hours at a pressure of 1.8 atmospheres in a pressure receptacle in an aqueous caustic soda liquor of 2° Bé. strength containing one gram of sodium myristyl-deca- or cetyl-dodeca- or stearyl-dodeca-glycoloxyacetate per liter. The material is then washed and dried. Even after repeated washings, the material still has outstanding wettability.

*Example 9*

A piece of unboiled cotton cretonne is boiled-off for two hours in an aqueous caustic soda liquor of 2° Bé. strength in a goods to bath ratio of 1:40 and in an open vessel, with the addition to the liquor of 0.5 gram of sodium oleyldodecaglycoloxyacetate per liter of liquor, after which the material is rinsed and dried. In contrast to a piece of this fabric which was boiled-off in the absence of the assistant, the treated piece can, in the padding process, by virtue of rapid and very uniform wettability, be excellently padded on the Foulard with a conventionally prepared vat-acid solution of dyestuff No. 1270 (Schultz, Farbstofftabellen, 7th edition, 1931), the dyestuff penetrating the material to be dyed in outstanding manner and the resulting dyeing being very even.

*Example 10*

A piece of unboiled cotton cretonne is boiled-off for two hours in an aqueous caustic soda liquor of 2° Bé. strength in a goods to bath ratio of 1:40 in an open vessel with the addition to the liquor of 0.75 gram of sodium oleyldodecaglycoloxyacetate per liter of liquor, after which the material is washed neutral and dried. Upon padding this material with a 1% by weight dyestuff solu-

tion of dyestuff No. 513 (Schultz, Farbstofftabellen, 7th edition, 1931), very uniform wetting is obtained and, upon completion of the dyeing, the material is very well through-dyed.

*Example 11*

Linen yarn is boiled-off first for two hours in an aqueous solution of 5 grams of calcined sodium carbonate and 0.2 gram of sodium oleyl-dodecaglycoloxyacetate per liter, and then subjected to the action of chlorine for one hour in the cold in a solution containing 5 grams of active chlorine per liter, acidified, aftertreated with sodium bisulfite, and dried. In this way, an outstandingly absorptive and dyeable yarn is obtained, whereas linen yarn treated in the same manner in the absence of the assistant has only a very slight absorptive capacity.

*Example 12*

A difficultly and non-uniformly wettable and swelling viscose fabric is boiled-off for one and one-half hours in a goods to bath ratio of 1:30 in a bath containing 1.0 gram of sodium oleyl-dodecaglycoloxyacetate and 0.5 gram of a 30% aqueous caustic soda solution per liter, after which the material is rinsed and dried. The so-treated fabric is wetted and swells much more uniformly than the same fabric which has been boiled-off without assistant.

*Example 13*

A piece of cotton cretonne fabric, as it comes from the loom, is boiled-off for two hours in a goods to bath ratio of 1:40 in an aqueous caustic soda liquor to 2° Bé. strength in an open vessel, with the addition to the bath of one gram of sodium oleyl-dodecaglycoloxyacetate per liter of liquor, after which the material is rinsed until it is neutral and then bleached in the cold for two hours with a bleaching liquor which contains one gram of active chlorine per liter, then acidified, dechlorinated with sodium bisulfite, and dried. The thus-treated fabric is, in comparison with like material which has been treated without an assistant, much whiter.

*Example 14*

Gray cotton pearl yarn 3/2 is boiled-off for two hours in an aqueous caustic soda liquor of 20 Bé. strength in a goods to bath ratio of 1:20 in an open vessel, with addition of one gram of sodium oleyl-dodecaglycoloxyacetate per liter of liquor, after which the yarn is washed neutral and dried. This yarn is then treated for one hour, in the mercerized or unmercerized state, in a chlorine bleaching bath containing one gram of active chlorine per liter, whereupon it is acidified, dechlorinated and then treated in an oxygenic bleaching bath which contains 10 milliliters of hydrogen peroxide (30%) and 1 milliliter of aqueous caustic soda solution (36° Bé.) per liter. The temperature is raised, in this connection, from 40° to 75° C. in the course of two hours and, after a temperature of 75° C. is reached, maintained at one hour between 75° and 80° C. The material is then rinsed and dried. In this way, a very nice bleached yarn is obtained, whereas a pearl yarn which is similarly treated but without the assistant according to this invention has, after being bleached, a considerably inferior white appearance.

It will be evident from the foregoing examples that the treatment according to the present invention is generally carried out at the boiling temperature of the aqueous alkaline treating bath, i. e. at a temperature above 75° C. However, for the sake of completeness, it may be noted that the treatment may be carried out at temperature within the range from 75° to 140° C.

While, as is evident from the foregoing illustrative examples, it is preferred to use the assistant (I) in the form of the sodium salt, such assistant may also with essentially equal success be used in the form of the acid or of other soluble salts, for instance potassium, ammonium and 75 amine salts of the acid.

<sup>1</sup> Similar results may be obtained with sodium tetramethyl nonyloctaglycoloxyacetate prepared from tetramethylnonanol (Enjay Co., Inc., New York).

The preferred aqueous alkaline treating bath is preferably constituted by a caustic soda liquor of 2° Bé. strength, but the invention may with equal success be carried out with other alkaline boiling-off or bucking baths, such as baths which density may vary from 0.5 to 10° Bé. and which instead of caustic soda contain caustic potassium or sodium carbonate or potassium carbonate.

The preferred concentration of assistant in the treating bath is 0.2 to 1 gram per liter, but in some cases it may be favorable to reduce or to increase the quantity of the assistant within the range of 0.1 to 10 grams per liter.

Having thus disclosed the invention, what is claimed is:

1. A bucking process for cleaing gray cellulose fibers, which comprises washing the gray cellulose fibers at temperatures of 75 to 140° C. with an aqueous alkaline solution of 0.5 to 10° Bé. containing as the essential alkaline ingredient a member selected from the group consisting of caustic soda, caustic potash, sodium carbonate and potassium carbonate, and as another essential ingredient a compound of the formula



wherein R is a member selected from the group consisting of saturated and unsaturated aliphatic hydrocarbon radicals containing 8 to 20 carbon atoms, and alkylphenyl and hydrogenated alkylphenyl radicals containing a total of 8 to 25 carbon atoms, n is a whole number which is 2 to 20, and M represents a cation selected from the group consisting of hydrogen, an alkali metal and ammonium, until impurities have been removed from the fibers and the latter have been rendered hydrophilic.

2. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient a member selected from the group consisting of caustic soda, caustic potash, sodium carbonate and potassium carbonate, and as another essential ingredient a compound of the formula



wherein R is a saturated aliphatic hydrocarbon radical containing 8 to 20 carbon atoms, n is a whole number which is 2 to 20, and M represents a cation selected from the group consisting of hydrogen, an alkali metal and ammonium, until impurities have been removed from the fibers and the latter have been rendered hydrophilic.

3. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient a member selected from the group consisting of caustic soda, caustic potash, sodium carbonate and potassium carbonate, and as another essential ingredient a compound of the formula



wherein R is an unsaturated aliphatic hydrocarbon radical containing 8 to 20 carbon atoms, n is a whole number which is 2 to 20, and M represents a cation selected from the group consisting of hydrogen, an alkali metal and ammonium, until impurities have been removed from the fibers and the latter have been rendered hydrophilic.

4. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient a member selected from the group consisting of causic soda, caustic potash, sodium carbonate and potassium carbonate, and as another essential ingredient a compound of the formula



wherein R is an alkylphenyl radical containing a total of 8 to 25 carbon atoms, n is a whole number which is 2 to 20, and M represents a cation selected from the group consisting of hydrogen, an alkali metal and ammonium, until impurities have been removed from the fibers and the latter have been rendered hydrophilic.

5. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient a member selected from the group consisting of caustic soda, caustic potash, sodium carbonate and potassium carbonate, and as another essential ingredient a compound of the formula



wherein R is a hydrogenated alkylphenyl radical containing a total of 8 to 25 carbon atoms, n is a whole number which is 2 to 20, and M represents a cation selected from the group consisting of hydrogen, an alkali metal and ammonium, until impurities have been removed from the fibers and the latter have been rendered hydrophilic.

6. A buckling process for cleaning gray cellulose fibers, which comprises washing the gray cellulose fibers at temperatures of 75 to 140° C. with an aqueous alkaline solution of 0.5 to 10° Bé. containing as the essential alkaline ingredient caustic soda and as another essential ingredient sodium lauryl-hexaglycoloxyacetate, until impurities have been removed from the fibers and the latter have been rendered hydrophilic.

7. A buckling process for cleaning gray cellulose fibers, which comprises washing the gray cellulose fibers at temperatures of 75 to 140° C. with an aqueous alkaline solution of 0.5 to 10° Bé. containing as the essential alkaline ingredient caustic soda and as another essential ingredient sodium myristyl-decaglycoloxyacetate, until impurities have been removed from the fibers and the latter have been rendered hydrophilic.

8. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient caustic soda and as another essential ingredient sodium cetyl-dodecaglycoloxyacetate, until impurities have been removed from the fibers and the latter have been rendered hydrophilic.

9. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient caustic soda and as another essential ingredient sodium stearyl-dodecaglycoloxyacetate, until impurities have been removed from the fibers and the latter have been rendered hydrophilic.

10. A bucking process for cleaning gray cellulose fibers, which comprises washing the gray cellulose fibers at temperatures of 75 to 140° C. with an aqueous alkaline solution of 0.5 to 10° Bé. containing as the essential alkaline ingredient caustic soda and as another essential ingredient sodium oleyl-dodecaglycoloxyacetate, until impurities have been removed from the fibers and the latter have been rendered hydrophilic.

#### References Cited in the file of this patent

#### UNITED STATES PATENTS

2,183,853 Hausmann et al. ----- Dec. 19, 1939  
2,340,977 Nusslein et al. ----- Feb. 8, 1944

#### OTHER REFERENCES

Hall: American Dyestuff Reporter, Jan. 2, 1933, pages 1-4.

U. S. DEPARTMENT OF COMMERCE  
PATENT OFFICE  
**CERTIFICATE OF CORRECTION**

Patent No. 2,802,715

August 13, 1957

Kurt Hofer et al.

It is hereby certified that error appears in the printed specification of the above numbered patent requiring correction and that the said Letters Patent should read as corrected below.

Column 1, line 24, for "state" read -- stated --; line 37, for "rinsed ro" read -- rinsed or --; column 3, line 46, for "dired" read -- dried --; column 4, line 31, for "liquor to" read -- liquor of --; line 68, for "temperature" read -- temperatures --; column 5, line 13, for "cleaing" read -- cleaning --; column 6, lines 24 and 32, for "buckling", each occurrence, read -- bucking --.

Signed and sealed this 25th day of February 1958.

(SEAL)

Attest:

KARL H. AXLINE  
Attesting Officer

ROBERT C. WATSON  
Commissioner of Patents